

## UNITED STATES PATENT OFFICE

MARVIN J. UDY, OF NIAGARA FALLS, NEW YORK

## PROCESS OF MAKING CHROMIC ACID

No Drawing.

Application filed November 5, 1925. Serial No. 67,152.

The invention is a process of making chromic acid.

In accordance with my invention chromic acid is prepared electrolytically by oxidizing chromic hydroxide in an electrolyte containing chromic acid while maintaining the composition of the electrolyte throughout the space between the electrodes substantially uniform.

10 It has been proposed heretofore to oxidize chromic hydroxide to chromic acid in a cell containing a porous diaphragm to separate the electrolyte surrounding the cathode from that surrounding the anode and to keep the 15 chromic acid formed away from the vicinity of the cathode. According to this prior process the electrolyte in the cathode compartment consists initially of sulfuric acid or a soluble sulfate, and the electrolyte in the 20 anode compartment consists initially of a suspension of chromic hydroxide in water slightly acidified with sulfuric acid or containing a soluble sulfate. As this process has been conducted, a product containing not over 10% 25 of  $\text{CrO}_3$  has been obtained.

I have found that little or no reduction of chromic acid takes place at the cathode if an electrolyte containing chromic acid is used and the cathode is immersed directly therein. 30 I have also found that when chromic hydroxide is added to a chromic acid solution it dissolves quite readily therein. Accordingly, by using a chromic acid electrolyte, the use of a diaphragm separating the cell into two 35 compartments may be dispensed with. It is also possible to produce either intermittently or as a continuous process a relatively concentrated chromic acid solution substantially free from impurities.

40 According to the preferred form of my invention, chromic hydroxide,  $\text{Cr}(\text{OH})_3$ , preferably freshly prepared and in a moist condition, is fed to an electrolytic bath consisting of an aqueous solution of chromic acid. The rate of feed should be as even as possible and such as to maintain the voltage .5 to 1.0 volt higher than that characteristic of the operation when no chromic hydroxide is present. The chromic hydroxide dissolves in the chromic acid solution, presumably as the result of a chemical

reaction in which chromium chromate is formed according to the following equation:



The oxidation of the chromate at the anode may be represented by the following equation:



The current density may be varied from a fraction of an ampere to 300 amperes per sq. ft., but the best results are obtained when operating within the range 100 to 200 amperes per sq. ft. It is preferred to maintain the temperature of the bath at from 95° C. to 100° C. I prefer to use a lead anode and a cathode of aluminum, iron or other suitable metal. The anode is preferably of the hollow type to permit of the circulation of steam or hot water through it to maintain the temperature of the bath within the limits specified.

The concentration of chromic acid in the electrolyte preferably should be maintained between 15 and 30%. When the operation is carried out as a continuous process, chromic acid should be withdrawn at such rate as to maintain the concentration of the electrolyte within the limits specified. According to this invention a product consisting of an aqueous solution having a  $\text{CrO}_3$  concentration of from 20 to 30% is regularly obtained, while higher concentrations may be obtained if desired.

The product consists of a substantially pure chromic acid solution which may be used without recrystallization for many purposes requiring pure chromic acid. A high current efficiency is obtained.

Best results are obtained by the use of chromic acid electrolyte free from mineral acids, although the process may be carried out with sulfuric acid present in small amounts not exceeding about one-half of one per cent.

I claim:

1. Process of making chromic acid which comprises passing current between an insoluble anode and a cathode in contact with an electrolyte containing trivalent chromium between approximately 15% and 30%  $\text{CrO}_3$ , the composition of the electrolyte through-

out the space between the electrodes being substantially uniform.

2. Process of making chromic acid which comprises passing current between an insoluble anode and a cathode in contact with an electrolyte containing between approximately 15% and 30%  $\text{CrO}_3$ , adding trivalent chromium to the electrolyte, and converting the trivalent chromium into chromic acid by anodic oxidation.
- 10 3. Process of making chromic acid which comprises passing current between an insoluble anode and a cathode in contact with an electrolyte containing between approximately 15% and 30%  $\text{CrO}_3$ , adding chromic hydroxide to the electrolyte, and converting the chromic hydroxide into chromic acid by anodic oxidation.
- 20 4. Process of making chromic acid which comprises passing current between an insoluble anode and a cathode in contact with an electrolyte consisting principally of an aqueous solution of hexavalent chromium, maintaining the composition of the electrolyte throughout the space between the electrodes substantially uniform, adding trivalent chromium to the electrolyte and converting the trivalent chromium into chromic acid by anodic oxidation.
- 30 5. Process of making chromic acid which comprises passing current between an insoluble anode and a cathode in contact with an electrolyte consisting principally of an aqueous solution of chromic acid, maintaining the composition of the electrolyte throughout the space between the electrodes substantially uniform, adding trivalent chromium to the electrolyte and converting the trivalent chromium into chromic acid by anodic oxidation.
- 40 6. Process of making chromic acid which comprises passing current between an insoluble anode and a cathode in contact with an electrolyte consisting principally of an aqueous solution of chromic acid and trivalent chromium, maintaining the composition of the electrolyte throughout the space between the electrodes substantially uniform, converting the trivalent chromium into chromic acid by anodic oxidation, continuously removing chromic acid, and adding water and trivalent chromium so as to maintain the concentration of the electrolyte within predetermined limits.

55 In testimony whereof, I affix my signature.  
MARVIN J. UDY.